

## UNITED STATES PATENT OFFICE.

CARL WILHELM SÖDERBERG, OF OSLO, NORWAY, ASSIGNOR TO DET NORSKE AKTIE-SELSKAB FOR ELEKTROKEMISK INDUSTRI OF NORWAY, OF OSLO, NORWAY.

## ELECTRODE MASS FOR SELF-BAKING ELECTRODES.

No Drawing. Application filed July 22, 1924, Serial No. 727,597, and in Norway July 25, 1923.

The present invention relates to the so-called continuous electrodes, which are baked in the electric furnace in which they are used and the object of the invention is 5 to provide an improved electrode mass from which an electrode is obtained having first class mechanical and electric qualities.

The usual carbon electrodes for electro-thermic use are, as is known, made by mix- 10 ing anthracite, previously heated to a red heat, cinders and other carbon materials with a binder, comprising pitch with some oil, or tar and pitch, to form a mass which is pressed or tamped into moulds. The elec- 15 trodes thus formed are then baked in special baking furnaces where they are slowly heated until the binder is coked, usually to 1100° C.

It is well known that good electrodes are 20 essential to an electric smelting furnace. Much work has been done in the effort to find the best methods for the production of electrodes and the following fundamental rules, which must be followed to obtain a 25 first class result, have been established:

1. The raw electrode should contain the least possible amount of volatile constituents. The less volatile constituents there are contained in the electrode mass, the 30 higher will be the specific gravity of the electrode.

2. The moulding of the electrode must be effected by means of high pressures or powerful blows whereby the particles of the 35 mass are pressed together and the air contained is driven out.

The method which is usually employed and which is considered to be the best is to 40 press the electrodes in hydraulic presses, employing pressures of about 300 kg. per square centimeter. The electrode mass is subjected to this high pressure for a long time and thereby the particles of the mass are displaced relatively to each other and 45 the air is driven out.

Also by tamping one has been able to 50 make good electrodes. The process then consists in subjecting the electrode mass to a tamping by means of a ram-like tamping apparatus. Both with regard to the trans- 55 portation and the baking of the raw electrodes and to make the mechanical treatment of the mass effective the electrode mass must have a definite consistency. It must as it is termed be able to "take pressing" and "take tamping". The mass must be treated mechanically in such a way that a solid and non-elastic electrode block results which shows a specific gravity corresponding to that which it is desired to obtain in the finished electrodes.

Applicant has, however, found that the mass which is used in the production of the so-called selfbaking electrodes must have a consistency quite different from usual mass to give a satisfactory result, it being usually impossible to employ high pressures for pressing the mass, or powerful tamping. Only a light tamping may be used, effected either manually or by means of small pneumatic tamping devices. If it is attempted to tamp usual electrode mass in this way it will not be possible to force the mass sufficiently together and an electrode results with lower specific gravity than usual electrodes, and the coherence and electric conductivity will be bad. This has the effect, that the electrodes stand less current density than first class electrodes and may in many cases lead to breakage, the electrodes not being strong enough to stand the strains to which they will be subjected. This behaviour is especially noticeable in the production of selfbaking electrodes which are provided with an iron- or metal armature. Such electrodes generally consist of an iron mantle with inwardly directed radial longitudinal ribs and this armature encloses the electrode mass and determines its form. In the lower part of the armature facing the furnace the electrode mass will be ready baked, in the upper part it is entirely raw.

The ribs transmit the current from the electrode holder to the baked part of the electrode and hold this tight for which reason they are provided with projections or the like which prevent the hard baked electrode from moving relatively to the ribs. Such a continuous electrode is generally 4 to 7 meters long.

Even if in using ordinary electrode mass for such electrodes it is possible by extremely accurate tamping to reach the right specific gravity of the electrode, the resulting electrodes will nevertheless not be so reliable as desired. When subjected to special strains electrode breakage may occur. The electrode divides up in pieces of 30 to 90 centimeters length which fall into the furnace when the iron armature is melted away.

The reason for this is that the electrode mass during the tamping gradually hardens as the carbon particles are worked together. The resulting hard non-electric mass is fixed relatively to the ribs of the iron armature which it envelops and to the other parts of the iron armature. As the electrode is consumed in the smelting furnace the armature is moved slowly downwards together with the electrode mass. A little above the furnace the electrode is heated to baking temperature and the mass shrinks, the binder being coked. The iron armature, however, expands on account of the rise in temperature and the electrode mass fixed to the armature is subjected to a strain which may result in a division of the electrode into pieces whose length varies with the electrode diameter and temperature conditions.

I have now found that the difficulties heretofore pointed out may be overcome by giving the mass a consistency with sufficiently low viscosity to allow the mass to settle during the heating in the electrode. To reach the right specific gravity and corresponding electric conductivity and mechanical qualities the mass must during the baking make a slow settling possible. The baking takes place in a mass subjected to pressure from the column of mass above. I obtain a suitable consistency by increasing the content of liquid constituents in the mass. The ordinary electrode mass for large electrodes generally contains a mixture of tar and pitch (for instance in the proportion 3 tar: 1 pitch) constituting 10 to 11% of the mass and is then easily tamped to a hard mass. If now the amount of tar-pitch is increased the mass will become more sticky at the tamping temperature and consequently difficult to treat with the tamping machine. At 18 to 22% tar-pitch it cannot be tamped at all. The treatment of one part of the surface of the mass with a machine for instance a pneumatic tamper with point only results in pressing down this part of the surface and raising the others. The consistency of the mass is that of a dough and the object of the tamping is in this case not to beat the mass together to attain a high specific gravity as in the case of ordinary pressed or tamped electrodes but only to bring the single portions of mass into intimate contact with each other and remove greater air bubbles.

My investigations have shown that such a mass has at the lower part of the continuous electrodes a considerably higher specific gravity than newly tamped mass in the upper part of the electrode. Samples of a ready baked electrode taken out from the lower end of a selfbaking electrode have the same specific gravity as the best pressed electrodes of the trade. This shows that a slow settling of the mass takes place while

it is in the electrode subjected to heat from the smelting furnace and charged with the weight of the mass above.

The difference between "tampable" and "non-tampable" mass is very apparent. Tampable mass subjected to a series of blows from a tamper becomes harder at each blow. At last the tamper strikes the mass with a sound as if striking a perfectly solid, non-elastic body. In a non-tampable mass such solidity is never obtained. In order to make clear how the change in consistency takes place when increasing the amount of liquid binder I have carried out comparative measurements of viscosity in a series of mixtures of finely pulverized anthracite and a liquid binder. The viscosity was determined by noting the number of seconds required for a rod of definite weight to move through a layer of mass of definite thickness. The results are given below:

At 24% binder the movement of the rod was not noticeable.

At 25% binder the movement of the rod was noticeable, but the time required was more than 1 hour.

At 26% binder the movement of the rod was a little quicker, but the time required was still more than 1 hour.

At 27% binder time still more than 1 hour.

Amount of binder: 27.5%, 28%, 28.5%, 29%, 30%, 32%.

Time required: 760, 100, 65, 58, 39, 20 seconds.

If the results are entered into a curve it will be seen, that the curve makes a sharp turning at 27.5 to 28% binder. This sudden change in the movability of the mass apparently corresponds to such a content of liquid that the solid carbon particles of the mass are no longer directly in touch with each other, but slide on the "lubricant", the binders used in electrode production being at the same time excellent lubricants.

The absolute percentage at which the mass ceases to be tampable depends on the amount of fine particles in the electrode mass and on the nature of the fines, and can therefore not be determined beforehand. In the investigations referred to above the "turning point" of the curve was found to be at 27.5% binder. This is of course only the case in a mixture of definite fines with a definite binder. If the quality or fineness of the fines are altered the "turning point" will become displaced. Under all circumstances, however, a curve for the viscosity is obtained giving a "turning point" at the content of binder at which the mass becomes noticeably "liquid".

In electrode mass for big electrodes generally  $\frac{1}{3}$  coarse particles are employed, that is a carbon material, for instance heated anthracite, in form of pieces having the size of a nut,  $\frac{2}{3}$  of the mass being fines and

binders. The coarse particles require very little binder to become moistened. The pieces are in the mass completely surrounded by fines on all sides and the consistency of the fines determines that of the mass. Practical experiments on a great scale now show, that the characteristic change in consistency by employment of the same material as in the experiments previously referred to, but with about  $\frac{1}{3}$  of coarse particles takes place at about 18% binder, and at 20% the mass is very movable. These figures are in good accordance with those found above it being considered that  $\frac{1}{3}$  of the mass requires very little binder. If more coarse particles are employed the change takes place at a lower content of binder. The mass is always treated in warm condition, generally at temperatures ranging from 60 to 100° C. The mixture of binders used in practice is then liquid.

By making the content of volatile constituents and binder in the mass sufficiently high tamping of the mass may be avoided altogether and the production of the continuous electrodes more takes the character of a casting. But also in such cases an excellent conductivity and specific gravity is attained in the finished electrodes, this being due to the exceedingly favorable baking conditions.

As mentioned above the iron mantle moves slowly downwards together with the electrode mass towards the crater of the furnace, the temperature of the mass rising slowly from about 60° C. to a bright red heat at the point of the electrode. At about 200° C. the first distillation of the most volatile constituents of the mass begins and these escape in the form of vapor. At about 700° C. the binders are transformed to high-molecular carbon compounds which are slowly transformed to a gradually harder coke. Thereby the porosity of the electrode is increased. The raw mass during the tamping still contains some air, but during the storing in the electrode a part of the air escapes and the porosity sinks to about 5%. In the completely baked electrode it is about 15 to 20%. I have found that during the distillation and coking the excess of binder will together with the distillation products try to escape downwards through the already baked and consequently most porous part of the electrode, but as just this part is heated to a red heat new amounts of carbon-hydrogen compounds will here continually be reduced, coke being formed and deposited in the pores of the electrode. The carbon particles consequently become further bound together, and the weight and conductivity of the electrode increases.

The foregoing detailed description has been given for clearness of understanding

only and no undue limitation should be deduced therefrom but the appended claims should be construed as broadly as permissible in view of the prior art.

What I claim as new and desire to secure by Letters Patent of the United States is:

1. An electrode mass for use in forming continuous electrodes, containing an excess of binder in proportions sufficiently high to cause the mass in warm condition to settle in the electrode. 75

2. An electrode mass for use in forming continuous electrodes, in which the proportion of binder content is sufficiently high to render the mass elastic and non-tampable. 75

3. An electrode mass for use in forming continuous electrodes, in which the proportion of binder content is sufficiently high to prevent reduction of the total volume of the mass under a tamping action. 80

4. An electrode mass for use in forming continuous electrodes, in which the proportion of binder content is sufficiently high to render the mass liquid. 85

5. An electrode mass for use in forming continuous electrodes, in which the binder content forms at least 14% of the mass. 90

6. The process of forming an electrode baked in the furnace in which it is used, and including an enclosing mantle comprising the steps of forming an electrode mass having a binder content sufficiently high to render the mass elastic and non-tampable and then casting the mass within the enclosing mantle of the electrode. 95

7. The process of forming an electrode baked in the furnace in which it is used and including an enclosing mantle comprising the steps of forming an electrode mass having a binder content sufficiently high to render the mass liquid, and then casting the mass within the enclosing mantle of the electrode. 100

8. The process of forming an electrode baked in the furnace in which it is used, and including an enclosing mantle comprising the steps of forming an electrode mass having a binder content of at least 14% of the mass and then casting the mass within the enclosing mantle of the electrode. 110

9. An electric furnace electrode of the kind which is baked during its use in any electric furnace characterized by a baked portion at the operating end and by soft electrode paste at the feeding end, said paste being of such consistency as automatically to exert sufficient pressure by its own weight to assure such compactness of the electrode materials throughout the baked portion of the electrodes as to afford physical and electrical characteristics of a pre-baked electrode. 115

CARL WILHELM SÖDERBERG.